

## UNITED STATES PATENT OFFICE

2,222,621

## ALLOY STEEL ARTICLE

Vsevolod Nicholas Krivobok, Pittsburgh, Pa., assignor to Rustless Iron and Steel Corporation, a corporation of Delaware

No Drawing. Original application June 25, 1935, Serial No. 28,374. Divided and this application October 19, 1937, Serial No. 169,906

1 Claim. (Cl. 138—47)

This application is a division of my copending Application 28,374 filed June 25, 1935 and entitled Alloy and manufactures, now Patent 2,125,929 of August 9, 1938, and the invention relates to 5 chromium-nickel alloy irons and steels and to tubular articles and manufactures of the same.

Among the objects of my invention is the production of chromium-nickel alloy irons and steels which are strong, tough, durable and which are 10 readily workable, as by forging and rolling into plates, bars, sheet, strip, rods and wire, which may be further machined, worked or formed, as by drilling, cutting, turning and bending, which may be welded where desired, to achieve a great 15 number of products, articles or manufactures, such as tubing and piping, fluid valves, all for high temperature duty, as in stills, evaporator units and the like, for semi-chemical uses in the canning, dairy, oil and photographic film industries, or in chemical calciners used in the 20 production of paints and dyes, or like articles, products or manufactures for high temperature service applications.

The invention accordingly consists in the combination of elements, composition of ingredients and mixture of materials, and in the articles, products and manufactures of the same, as described herein, the scope of the application of which is indicated in the following claim.

As conducive to a clearer understanding of certain features of my invention it may be noted at this point that the austenitic chromium-nickel irons and steels (irons and steels containing approximately, 10 to 25% chromium, 7% to 15% nickel, and the balance substantially iron) are used in the production of a wide variety of corrosion-resistant and mildly heat-resistant products or articles of manufacture. Thus, these austenitic irons and steels, especially the 18—8 irons and steels (irons and steels containing 18% chromium, 8% nickel, and the balance substantially iron) may be used in a number of interior or exterior architectural applications, such as decorative trim, ornamentation and fixtures. Likewise, these irons and steels may be employed for a variety of kitchen, soda fountain, dairy and hospital applications, as in cooking and serving utensils, containers and appliances, counter and furniture trim and the like, where permanently 40 bright corrosion-resistant metal capable of withstanding the corrosive action of various fruit and vegetable acids, is desired. Similarly, these irons and steels are widely adapted for various chemical plant apparatus and equipment where metal 45 resistant to the corrosive attack of acids, alkalis

and salts at room temperature, or slightly elevated temperatures, is required.

These austenitic chromium-nickel irons and steels, however, are not satisfactorily adaptable to extremely high temperature duty, especially high 5 temperature duty under strongly oxidizing or corrosive conditions, largely because of the susceptibility of these irons and steels to intergranular corrosion and because of their tending to flow at high temperatures.

One of the outstanding objects of my invention is the production of strong, tough and ductile alloy irons and steels, which may be readily worked or formed into a variety of tubular products, articles or manufactures, which are resistant to 10 scaling, pitting and intergranular corrosion or corrosion embrittlement, at high temperatures over long periods of continuous operation under a variety of corrosive or corrosion-fostering media and under the many varying conditions en- 15 countered in actual, practical use.

Referring now more particularly to the practice of my invention, alloy iron or steel analyzing approximately, 18% chromium, 8% nickel, 2.5% to 3.5% tungsten, 1% to 2% molybdenum, .07% to 25 .1% carbon, and the balance substantially iron, with the usual percentages of silicon, manganese, sulphur and phosphorus, is conveniently produced in an electric furnace in a suitable manner, as for example, as described in Patent No. 30 1,925,182 granted to Alexander L. Feild September 5, 1933 and entitled Process for the manufacture of rustless iron. The alloy iron or steel of desired analysis is poured into suitable ingot molds where it is permitted to cool. The formed 35 ingots are stripped from the molds and fashioned into blooms or billets in accordance with known methods and conveniently converted by hot-working methods or a combination of hot and cold methods into plate, sheet, strip, bars, rods or wire 40 of desired dimensions. When desired the converted products are annealed to relieve working strains and then cooled all in accordance with known methods. The cold-rolled sheet and strip, however, is preferably used without benefit of 45 annealing treatment in order to gain full realization of the strength, hardness and other superior physical characteristics imparted by the cold-working operations.

My alloy iron or steel is essentially austenitic 50 in structure but contains certain new constituents in the form of complex ferrites and carbides lending to the metal superior working, corrosion-resisting and physical characteristics. The metal is corrosion-resistant and heat-resistant, with- 55

standing the conditions of high temperature duty over long periods of continuous use and under a wide variety of corrosive or corrosion-fostering media, including sulphur-bearing vapors and gases, such as hydrogen sulphide, in addition to those agents normally present in the atmosphere, without general, local or intergranular corrosion, grain growth, fatigue or failure. For example, a bar of austenitic chromium-nickel iron analyzing 10 approximately, 18% chromium, 8% nickel, 3% tungsten, 2% molybdenum, 10% carbon, and the balance substantially iron, subjected to a stress of 8,000 pounds per square inch at a temperature of 1500° F., under ordinary atmospheric conditions, has a life of about 600 hours. Ordinary 18-8 chromium, 8% nickel, .07% carbon, and the balance substantially iron, has a life of only about 12 hours under like conditions of operation.

My chromium-nickel alloy iron or steel, in 20 addition to having a life under high temperature operating conditions greatly in excess of heretofore known and/or used chromium-nickel irons and steels, is strong, tough and ductile and readily lends itself to a variety of working and forming operations either from sheet, strip or bar stock. The metal may be forged, upset or drawn, it may be hot or cold rolled into sheet, strip and bar stock, which may be further worked or formed, as by bending, punching or blanking 25 and may be machined by drilling, cutting, threading or the like, followed by welding where desired, either with the oxy-acetylene torch or with the electric arc (preferably employing welding rods of approximately the same analysis as the stock welded) to achieve a great many tubular articles, products and manufactures. (The 30 various welded articles, products and manufactures are preferably given a stabilizing heat-treatment in accordance with well known methods to establish a stabilized condition of the metal after the welding is completed in order to assure minimum intergranular corrosion and maximum corrosion resistance in use.) For example, the bar, sheet and strip worked or formed 35 as above indicated is fashioned into tubes, fluid valves, couplings, all for high temperature duty as in boilers, condensers, oil cracking stills, evaporator units and the like, or for semi-chemical uses in the canning, dairy, oil and photographic film industries, or chemical calciners, as used in the production of iron-free chemicals, such as 40 paints and dyes.

Thus, it will be seen that there is provided in this invention a chromium-nickel alloy iron or steel and articles, products and manufactures of the same in which the various objects hereinbefore noted, together with many thoroughly practical advantages are successfully achieved. It will be seen that the alloy is strong, tough, 45

corrosion-resistant and heat-resistant and that it readily lends itself to a variety of working or forming operations into a number of commercial tubular articles, products or manufactures, many of which are set forth above, which are especially adapted to withstand continuous high temperature and high pressure duty over long periods of time and under the many varying conditions of actual, practical use, such as the wash and scour of corrosive fluids. 5

While as illustrative of my invention an austenitic chromium-nickel iron containing approximately, 18% chromium, 8% nickel, 2.5% to 3.5% tungsten, 1% to 2% molybdenum, .07% to .1% carbon, and the balance substantially iron, 10 is specifically described, good results are achieved where the chromium content ranges between 10% and 25% and the nickel content between 7% and 15%. Similarly, chromium-nickel alloy irons or steels possessing long life at high temperatures in combination with good mechanical workability, are achieved where the tungsten content ranges from just above 2% up to about 4% and the molybdenum content ranges from about .7% up to about 3%. Likewise, good high 15 temperature duty characteristics are achieved in modified chromium-nickel alloy irons and steels where the carbon content ranges between .03% and .2%. 20

Certain further benefits in long-life alloy iron 30 and steel at unusually high operating temperatures are achieved by adding to the tungsten-molybdenum-chromium-nickel alloy iron or steel, the further ingredient, manganese, in the amount of from about .5% to 3%. High temperature 35 duty irons and steels of this analysis are especially resistant to the corrosive attack of sulphur-bearing gases at high temperatures and are of somewhat improved workability over the high temperature irons and steels indicated above. 40

As many possible embodiments may be made of my invention and as many changes may be made in the embodiment hereinbefore set forth, it is to be understood that all matter described herein 45 is to be interpreted as illustrative, and not in a limiting sense. 45

I claim:

Wrought alloy austenitic 10 to 25 per cent chromium, 7 to 15 per cent nickel and .03 to .20 per cent carbon, stainless steel tubular articles characterized by their freedom from corrosion embrittlement and by their resistance to the wash and scour of corrosive fluids, used under conditions of high internal pressures and at high temperatures, said characteristics being produced by the inclusion in said alloy steel of .7 to 3 per cent molybdenum and over 2 per cent up to 4 per cent tungsten. 50 55

VSEVOLOD NICHOLAS KRIVOBOK.